

## UNITED STATES PATENT OFFICE

2,604,400

NAPHTHYL HYDRAZINE SULFONIC ACIDS  
IN DIRECT POSITIVE PHOTOGRAPHIC  
PROCESSES

Frederic R. Bean and Harold D. Russell, Rochester, N. Y., assignors to Eastman Kodak Company, Rochester, N. Y., a corporation of New Jersey

No Drawing. Application March 28, 1951,  
Serial No. 218,072

6 Claims. (Cl. 95—88)

1

This invention relates to photography and particularly to a method of making direct positive photographs.

In Fallesen U. S. Patent 2,497,875, a method is described for making direct positive photographs with an internal latent image type emulsion by developing the exposed emulsion in an aerial fogging developer with access of oxygen.

Ives U. S. application, Serial No. 192,380, filed October 26, 1950, now Patent No. 2,588,982, describes a method for developing direct positive images in an exposed internal latent image emulsion by the use of hydrazine or certain hydrazine derivatives so that no special aeration technique for production of the positive image is required.

We have found that naphthyl hydrazine sulfonic acids may be used in the developer or emulsion to develop direct positive images in an internal latent image emulsion. These compounds are relatively non-toxic and produce satisfactory direct positive images without the addition of oxidizing agents to the developer or the use of any special aeration method.

The photographic emulsion used in the process of our invention is a gelatino-silver halide emulsion such as a silver bromide emulsion, a silver bromoiodide emulsion or a silver chloroiodide emulsion. It need not contain optical sensitizing dyes although certain sensitizing dyes may be added to it for the purpose of optical sensitizing or for promoting reversal. The emulsion should be undigested or if digested, the digestion should be carried out without the use of sulfur sensitizers. An emulsion of this type is that known as Burton's emulsion, described in Wall, "Photographic Emulsions," 1929, pages 52 and 53. Burton's emulsion is made as follows:

A. Silver nitrate----- 100  
Water ----- 500  
Ammonia—to form clear solution.  
B. Potassium bromide----- 80  
Potassium iodide----- 50  
Soft gelatin----- 20  
Water ----- 1000  
C. Dry gelatine----- 250

B. is heated to 70° C. and A. cold, added to B with constant shaking, digested for 20 minutes at 50° C., and allowed to cool slowly. C. is added after being allowed to swell for 20 minutes in water, drained and melted. The emulsion is then set and washed.

An internal latent image emulsion, that is, one which forms the latent image mostly inside the silver halide grains, as described on pages 296

and 297 of Mees' "The Theory of the Photographic Process," 1942, is especially useful for the process of our invention.

Most of the internal latent image emulsions are silver bromoiodide emulsions of high iodide content, preferably containing at least 10%—20% of iodide. Burton's emulsion is an emulsion of this type, having a silver iodide content of approximately 40% of the content of silver halide. It is not absolutely essential, however, for the emulsion to contain silver iodide.

An internal latent image emulsion made as described in Davey and Knott U. S. application Serial No. 82,914, filed March 22, 1949, now Patent No. 2,592,250, may also be used according to our invention. This emulsion is prepared by first forming in the absence of ammonia and in one or more stages silver salt grains consisting at least partly of a silver salt which is more soluble in water than silver bromide, subsequently converting the grains to silver bromide or silver bromoiodide and if the silver iodide content of the emulsion is less than 6% calculated on the total silver halide, treating such grains with an iodine compound to bring the silver iodide up to at least 6%, ripening preferably in the absence of ammonia and then either washing out some of the soluble salts or washing out the whole of the soluble salts, followed by the addition of soluble salts such as soluble chloride or bromide. An example of an emulsion made in this way is as follows:

## Solution No. 1

|                     |          |           |
|---------------------|----------|-----------|
| Inert gelatine----- | 20 grams | at 40° C. |
| KCl -----           | 20 grams |           |
| Water -----         | 560 cc.  |           |

## Solution No. 2

|             |           |           |
|-------------|-----------|-----------|
| KCl -----   | 100 grams | at 45° C. |
| Water ----- | 520 cc.   |           |

## Solution No. 3

|                         |           |           |
|-------------------------|-----------|-----------|
| AgNO <sub>3</sub> ----- | 195 grams | at 45° C. |
| Water -----             | 520 cc.   |           |

## Solution No. 4

|             |           |           |
|-------------|-----------|-----------|
| KBr -----   | 160 grams | at 45° C. |
| KI -----    | 40 grams  |           |
| Water ----- | 500 cc.   |           |

Run Solutions Nos. 2 and 3 simultaneously into Solution No. 1 in a vessel, taking 90 seconds to do this. Then ripen for 1 minute at 45° C. Next add 235 grams of inert gelatine (dry). Then ripen at 45° C. for 15 minutes during which

time the gelatine dissolves. Set and shred the emulsion and then wash until free from all soluble bromide and then add about 150 cc. of 10% solution of KCl (by weight), and then add water to make 3½ litres.

An internal latent image type of silver halide emulsion may be defined as one which, when a test portion is exposed to a light intensity scale for a fixed time between  $\frac{1}{100}$  and 1 second, and developed for 4 minutes at 20° C. in the ordinary, 10 "surface" developer (Example I), exhibits a maximum density not greater than  $\frac{1}{5}$  the maximum density obtained when the same emulsion is equally exposed and developed for 3 minutes at 20° C. in an internal type developer (Example II). 15 Preferably the maximum density obtained with the surface developer is not greater than  $\frac{1}{10}$  the maximum density obtained when the same emulsion is developed in the internal type developer. Stated conversely, an internal latent image emulsion, when developed in an internal type developer (Example II) exhibits a maximum density at least 5, and preferably at least 10, times the maximum density obtained when the same emulsion is exposed in the same way and developed in a surface developer (Example I).

Our process is carried out by exposing the internal latent image emulsion layer to an object or image and then placing the exposed emulsion layer directly in a silver halide developing solution containing one or more of the naphthyl hydrazine sulfonic acids, or by incorporating the naphthyl hydrazine sulfonic acid in the emulsion, and placing the exposed layer in a developing solution not containing the hydrazine compound. 30 Developing agents suitable for use in the process of our invention include the usual phenolic or aminophenol type developing agents such as N-methyl-p-aminophenol sulfate, hydroquinone, catechol, 2-methyl hydroquinone, 2-chlorohydroquinone, p-aminophenol, and pyrogallol. If the naphthyl hydrazine sulfonic acid is in the developing solution, the developing solution should have a pH of from 8.5 to 13 depending upon the degree of activity of the particular hydrazine 45 compound which it contains although the preferred range with most hydrazine compounds is from pH 10 to pH 12.

The following naphthyl hydrazine sulfonic acids are suitable for use according to our invention:



1-naphthyl hydrazine-6-sulfonic acid

1-naphthyl hydrazine-4-sulfonic acid  
(Beilstein 15, 645)

1-naphthyl hydrazine-7-sulfonic acid



4-bromo-1-naphthyl hydrazine-7-sulfonic acid



2-naphthyl hydrazine-7-sulfonic acid

2-naphthyl hydrazine-6-sulfonic acid  
(J. Prakt. Chem. 79, 369)2-naphthyl hydrazine-4,8-disulfonic acid  
(P. B. Report, No. 986, 330)2-naphthyl hydrazine-5,7-disulfonic acid  
(P. B. Report, No. 986, 330)

2-naphthyl hydrazine-6,8-disulfonic acid

An ordinary surface type developer, that is, one which develops an image only on the surface of the grains of an internal latent image emulsion is the following:

## Example I

|                                    | Grams |
|------------------------------------|-------|
| p-Hydroxyphenylglycine             | 10    |
| Sodium carbonate (crystals)        | 100   |
| Water to 1 liter.                  |       |
| Development time, 4 min. at 20° C. |       |

An internal type developer, that is, one which develops an image inside the grains of an internal latent image emulsion is the following:

## Example II

|                                       | Grams |
|---------------------------------------|-------|
| Hydroquinone                          | 15    |
| N-methyl-p-aminophenol sulfate        | 15    |
| 70 Sodium sulfite (anhydrous)         | 50    |
| Potassium bromide                     | 10    |
| Sodium hydroxide                      | 25    |
| Sodium thiosulfate (crystals)         | 20    |
| Water to 1 liter.                     |       |
| 75 Development time, 3 min. at 20° C. |       |

Our invention will be further illustrated by reference to the following specific examples:

*Example III*

An emulsion made as described in the Davey and Knott application Serial No. 82,914 was coated on a support, dried and exposed on an intensity scale sensitometer to 3000° Kelvin tungsten illumination and developed for from 1 to 5 minutes at 75° F. in a solution of the following composition:

|                                      | Grams |
|--------------------------------------|-------|
| N-methyl-p-aminophenol sulfate       | 5     |
| Hydroquinone                         | 10    |
| Sodium sulfite                       | 75    |
| Sodium hydroxide                     | 10    |
| 5-methyl benzotriazole               | 0.2   |
| 1-naphthyl hydrazine-6-sulfonic acid | 4     |
| Water to 1 liter.                    |       |

With these developing conditions a direct positive image of satisfactory characteristics was obtained.

*Example IV*

A portion of the same emulsion as that used in Example III was coated and exposed in the same way as Example III and was developed for from 1 to 5 minutes at 70° F. in a solution of the following composition:

|                                      | Grams |
|--------------------------------------|-------|
| Hydroquinone                         | 15    |
| Sodium sulfite                       | 75    |
| Sodium carbonate                     | 50    |
| Sodium hydroxide                     | 10    |
| 5-methyl benzotriazole               | 0.2   |
| 1-naphthyl hydrazine-6-sulfonic acid | 4     |
| Water to 1 liter.                    |       |

With these developing conditions a direct positive image of satisfactory characteristics was obtained.

*Example V*

A portion of the same emulsion as that used in Example III was coated and exposed in the same way as Example III and was developed for from 1 to 5 minutes at 70° F. in a solution of the following composition:

|                                      | Grams |
|--------------------------------------|-------|
| Pyrocatechol                         | 15    |
| Sodium sulfite                       | 75    |
| Sodium hydroxide                     | 15    |
| 5-methyl benzotriazole               | 0.2   |
| 1-naphthyl hydrazine-6-sulfonic acid | 3     |
| Water to 1 liter.                    |       |

With these developing conditions a direct positive image of satisfactory characteristics was obtained.

The incorporation of the naphthyl hydrazine sulfonic acids in the emulsion is illustrated by the following example:

*Example VI*

An emulsion was made as in Example III except that previous to coating, a quantity of 1-naphthyl hydrazine-7-sulfonic acid or a mixture of 1-naphthyl hydrazine-7-sulfonic acid and 1-naphthyl hydrazine-6-sulfonic acid was added in the ratios between 2 grams and 8 grams per gram mole of silver halide. The coatings were made with and without sensitizing dye. When the dried emulsions were ex-

posed and developed in the following solution a positive image was obtained:

|                                | Grams |
|--------------------------------|-------|
| N-methyl-p-aminophenol sulfate | 5     |
| Hydroquinone                   | 10    |
| Sodium sulfite                 | 75    |
| Sodium hydroxide               | 10    |
| 5-methyl benzotriazole         | 0.2   |
| Water to 1 liter.              |       |

Although the reversal effect obtained in our process does not require agitation of the developer or the presence of oxidizing agents, we believe that the fogging action obtained is related to aerial oxidation. The active agent, which is derived from the hydrazine compound appears to have a long life in the developing solutions and only brief exposures to atmospheric oxygen appear sufficient to produce fogging even in the absence of continued aeration. Our process, therefore, has distinct advantages for deep tank photographic processing.

1-naphthyl hydrazine-6-sulfonic acid was prepared as follows:

25 A warm solution of 67 parts of 1-naphthylamine-6-sulfonic acid in 450 parts of water and 10 parts of sodium hydroxide was treated with 46 parts of concentrated sulfuric acid, and the mixture cooled to 0° C. Fifty parts of ice were added, followed by 44 parts by volume of a 40 per cent solution of sodium nitrite. After the solution had been stirred in the cold for 2 to 3 hours the brown diazonium salt was removed by filtration and washed with cold water.

30 The salt was then added in portions to a cold (less than 10° C.) solution of 150 parts of stannous chloride dihydrate in 275 parts by volume of concentrated hydrochloric acid and 135 parts of water. The mixture was stirred overnight, filtered, and the white solid product washed thoroughly with water.

35 1-naphthyl hydrazine-7-sulfonic acid was prepared as follows:

40 A solution of 180 parts (0.6 mole) of the sodium salt of 1-naphthylamine-7-sulfonic acid (70-75 per cent pure) in 2400 parts of water was stirred with 25 parts of Nuchar and filtered. The filtrate was combined with 78 parts by volume of 40 per cent sodium nitrite solution, cooled to 15-20° C., and added in a fine stream during 3/4 of an hour to a cold solution of 93 parts of concentrated sulfuric acid in 500 parts of water. The temperature was maintained below 10° C., and the mixture stirred for 1 1/2 hours after the addition was complete. The solid diazonium salt was allowed to settle, and the clear mother liquor decanted. The dark brown solid was filtered and washed with a little cold water. It was made into a thin paste with water and added gradually (1/2 hour) to a cold solution (previously filtered through Filter Cel) of 300 parts of stannous chloride dihydrate in 550 parts by volume of concentrated hydrochloric acid and 275 parts of water. The reaction temperature was kept below 10° C. by an ice-salt bath and regulation of the rate of addition.

45 The thick tan slurry was stirred a while longer and allowed to stand overnight. It was filtered and washed thoroughly with water; this necessitates removal of the cake from the filter for each of two or three washes. The yield of gray product was about 70 parts (55 per cent).

4-bromo-1-naphthyl hydrazine-7-sulfonic acid was prepared in the same way as 1-naphthyl hydrazine-6-sulfonic acid, using 4-bromo-1-naph-

thylamine-7-sulfonic acid in place of 1-naphthylamine-6-sulfonic acid.

4-bromo-1-naphthylamine-7-sulfonic acid was prepared as follows:

A. 1-acetylamino-naphthalene-sulfonic acid

A mixture of 600 parts of technical 1-naphthylamine-7-sulfonic acid (sodium salt), 2500 parts of glacial acetic acid, 500 parts of acetic anhydride and 54 parts of sodium acetate was heated under reflux for 6 hours, cooled, and filtered. The filtrate was acidified with 300 parts by volume of concentrated hydrochloric acid, and the product filtered, washed with acetic acid, and dried. The yield consisted of 354 parts of material containing about 20% sodium chloride.

B. 4-bromo-1-naphthylamine-7-sulfonic acid

A solution of 324 parts of the 1-acetylamino-naphthalene-7-sulfonic acid in 1400 parts of glacial acetic acid containing 100 parts of sodium acetate was filtered, and the filtrate diluted with 2000 parts of acetic acid. Bromine (160 parts) was added dropwise to this solution at 35-40°. One hour later, the unused bromine was destroyed with sulfur dioxide, 82 parts of sodium acetate was added, and the mixture filtered.

Hydrolysis to the free amine was carried out by heating for 1½ hours on the steam bath with 800 parts of 6N hydrochloric acid. The 4-bromo-1-naphthylamine-7-sulfonic acid which separated (176 parts) was filtered, washed and dried.

2-naphthyl hydrazine-7-sulfonic acid and 2-naphthyl hydrazine-6,8-disulfonic acid were prepared in the same way as 1-naphthyl hydrazine-6-sulfonic acid, using respectively, 2-naphthylamine-7-sulfonic acid and 2-naphthylamine-6,8-disulfonic acid instead of 1-naphthylamine-6-sulfonic acid.

It will be understood that the examples and modifications included herein are illustrative only and that our invention is to be taken as limited only by the scope of the appended claims.

We claim:

1. The method of obtaining a direct positive image in a silver halide emulsion layer, which comprises exposing to light rays to which the emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the maximum density obtained when the equally exposed silver halide emulsion is developed for 4 minutes at 20° C. in the following surface developer (I):

|                        | Grams |
|------------------------|-------|
| p-Hydroxyphenylglycine | 10    |
| Sodium carbonate       | 100   |
| Water to 1 liter.      |       |

and developing only the unexposed portion of said emulsion layer in the presence of at least one naphthyl hydrazine sulfonic acid.

2. The method of obtaining a direct positive image in a silver halide emulsion layer, which comprises exposing to light rays to which the

emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the maximum density obtained when the equally exposed silver halide emulsion is developed for 4 minutes at 20° C. in the following surface developer (I):

|                        | Grams |
|------------------------|-------|
| p-Hydroxyphenylglycine | 10    |
| Sodium carbonate       | 100   |
| Water to 1 liter.      |       |

and developing only the unexposed portion of said emulsion layer in a developer containing at least one naphthyl hydrazine sulfonic acid.

3. The method of obtaining a direct positive image in a silver halide emulsion layer, which comprises exposing to light rays to which the emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the maximum density obtained when the equally exposed silver halide emulsion is developed for 4 minutes at 20° C. in the following surface developer (I):

|                        | Grams |
|------------------------|-------|
| p-Hydroxyphenylglycine | 10    |
| Sodium carbonate       | 100   |
| Water to 1 liter.      |       |

and developing only the unexposed portion of said emulsion layer in a developer containing 1-naphthyl hydrazine-7-sulfonic acid.

4. The method of obtaining a direct positive image in a silver halide emulsion layer, which comprises exposing to light rays to which the emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                |       |

gives a maximum density at least 5 times the

maximum density obtained when the equally exposed silver halide emulsion is developed for 4 minutes at 20° C. in the following surface developer (I) :

|                        | Grams | 5 |
|------------------------|-------|---|
| p-Hydroxyphenylglycine | 10    |   |
| Sodium carbonate       | 100   |   |
| Water to 1 liter.      |       |   |

and developing only the unexposed portion of said emulsion layer in a developer containing 1-naphthyl hydrazine-6-sulfonic acid.

5. The method of obtaining a direct positive image in a silver halide emulsion layer, which comprises exposing to light rays to which the emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II) :

|                                  | Grams |  |
|----------------------------------|-------|--|
| Hydroquinone                     | 15    |  |
| Monomethyl-p-aminophenol sulfate | 15    |  |
| Anhydrous sodium sulfite         | 50    |  |
| Potassium bromide                | 10    |  |
| Sodium hydroxide                 | 25    |  |
| Sodium thiosulfate               | 20    |  |
| Water to 1 liter.                |       |  |

gives a maximum density at least 5 times the maximum density obtained when the equally exposed silver halide emulsion is developed for 4 minutes at 20° C. in the following surface developer (I) :

|                        | Grams | 35 |
|------------------------|-------|----|
| p-Hydroxyphenylglycine | 10    |    |
| Sodium carbonate       | 100   |    |
| Water to 1 liter.      |       |    |

and developing only the unexposed portion of said emulsion layer in a developer containing 1-naphthyl hydrazine-6-sulfonic acid and 1-naphthyl hydrazine-7-sulfonic acid.

6. The method of obtaining a direct positive image in a silver halide emulsion layer, which comprises exposing to light rays to which the emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II) :

|                                  | Grams |  |
|----------------------------------|-------|--|
| Hydroquinone                     | 15    |  |
| Monomethyl-p-aminophenol sulfate | 15    |  |
| Anhydrous sodium sulfite         | 50    |  |
| Potassium bromide                | 10    |  |
| Sodium hydroxide                 | 25    |  |
| Sodium thiosulfate               | 20    |  |
| Water to 1 liter.                |       |  |

gives a maximum density at least 5 times the maximum density obtained when the equally exposed silver halide emulsion is developed for 4 minutes at 20° C. in the following surface developer (I) :

|                        | Grams |  |
|------------------------|-------|--|
| p-Hydroxyphenylglycine | 10    |  |
| Sodium carbonate       | 100   |  |
| Water to 1 liter.      |       |  |

and developing only the unexposed portion of said emulsion layer in a developer containing 4-bromo-1-naphthyl hydrazine-7-sulfonic acid.

FREDERIC R. BEAN.  
HAROLD D. RUSSELL.

No references cited.